

## UNITED STATES PATENT OFFICE

2,397,015

SILVER HALIDE PHOTOGRAPHIC  
EMULSIONS

John David Kendall and Douglas James Fry,  
Ilford, England, assignors to Ilford Limited,  
Ilford, England, a British company

No Drawing. Application January 13, 1944, Se-  
rial No. 518,106. In Great Britain February 12,  
1943

14 Claims. (Cl. 95—6)

This invention relates to silver halide photographic emulsions and particularly to gelatino silver chloride photographic emulsions such as are used in development papers for contact printing, i. e. the so-called "gaslight" printing papers.

It is well known that the colour of developed images obtained from gelatino silver chloride development emulsions can be controlled to some extent by the addition of certain substances to the emulsion or to the developer. In the absence of any special additions the developed images may vary from a greenish to a fairly neutral black. It is generally preferred that the developed images should be on the bluer side of neutral black rather than on the greener side, and various suggestions have hitherto been made for obtaining the desired blue-black images. Thus it is known to include in the emulsion a small quantity of a quinine salt, which has the effect of yielding developed images of a good blue-black colour. Various other substances have been suggested as emulsion additions for the same purpose, but none of those hitherto proposed is so satisfactory as the quinine salts. Many compounds have likewise been suggested as developer additions, but from both manufacturers' and users' standpoints, it is better to include the blue-black toning substance in the emulsion since the products can then be developed with standard developers.

According to the present invention silver chloride emulsions which yield images of excellent blue-black colour on development are obtained by including in the emulsion, during its manufacture, a quinoline compound of the general formula:



where R<sub>1</sub> is an alkyl or aralkyl group, R<sub>2</sub> is a hydrogen atom or an alkyl or aralkyl group, or R<sub>1</sub> and R<sub>2</sub> together form the residue of an alicyclic nucleus, and R<sub>3</sub> is a hydrogen atom or a lower alkyl group. These compounds may be further substituted in the carbocyclic ring and may be applied in the form of their mineral acid salts.

Thus the compounds employed are essentially 4-alkyl quinolines or 4-aralkyl quinolines which may or may not contain other substituent groups. It is found that any substituents may be present in the carbocyclic ring, e. g. halogen atoms, hydrocarbon groups or alkoxy, aryloxy or aralkyloxy groups, or benz groups fused to the carbocyclic ring, though lower alkyl substituents and lower alkoxy substituents are preferred. Compounds containing benz groups fused to the carbocyclic ring, e. g. in the 5:6- or 7:8-positions,

though operative, are generally less satisfactory than those without such groups.

The group R<sub>1</sub> may be any alkyl or aralkyl group, e. g. methyl, ethyl or higher alkyl, or benzyl. The group R<sub>2</sub> may be a hydrogen atom or any alkyl or aralkyl group as specified above. The group R<sub>3</sub> may be a lower alkyl group, but it is strongly preferred that it be a hydrogen atom, i. e. that the 2-position in the nitrogen ring should be unsubstituted. It is found that in general compounds of the above general formula in which R<sub>3</sub> is a lower alkyl group are less effective for the purposes of this invention than the corresponding compounds in which the 2-position is unsubstituted; for example, 2:4-dimethyl quinoline, though effective, is considerably less effective than 4-methyl quinoline.

Specific compounds which are of particular value are 4-methyl quinoline containing no other substituent group, and 4-methyl quinolines containing the following additional substituent groups: 3-methyl, 3-ethyl, 6-methyl, 7-methyl, 6-methoxy, 6-ethoxy, 8-ethoxy, and combinations of such groups. Other compounds of particular value are the corresponding compounds where the 4-methyl group is replaced by a 4-ethyl, 4-higher alkyl or 4-benzyl group. Particularly valuable compounds of the type where R<sub>1</sub> and R<sub>2</sub> in the formula form an alicyclic ring are 3:4-tetramethylene quinoline and corresponding compounds containing alkyl or alkoxy groups in the carbocyclic ring of the quinoline nucleus.

As indicated above, the compounds can be used either as the free bases or as mineral acid salts. Thus, for example, the compounds may be used as the hydrochlorides or bisulphates.

The proportion of compound added to the emulsion will depend on the particular compound used and on the precise nature of the emulsion. In general a good blue-black tone can be obtained using the compounds of this invention in proportions of the order of 25 ccs. of a 1% solution of the compound per pound of emulsion, though lower proportions or higher proportions can be used, e. g. of the order of 5 to 50 ccs. of a 1% solution per pound of emulsion.

Many substances when added to photographic emulsions have undesirable effects on the qualities of an emulsion, i. e. loss of speed, increased tendency to the formation of fog (i. e. developed silver not arising from the exposure) and on the contrast of the developed images. It is a particular merit of the compounds used as blue-black toners according to the present invention that they do not have any serious adverse effect in respect of any of these properties.

The following examples illustrate the invention:

## Examples

A gelatino silver chloride emulsion of the "gas-

"light" type was prepared and to portions of it were added proportions of different compounds according to this invention. A control sample containing quinine bisulphate as the blue-black toning agent was also prepared. The quinine bisulphate and other compounds were each added in the proportion of 25 ccs. of a 1% solution per pound of emulsion. The samples were coated on paper base, exposed, developed in a standard metol-hydroquinone developer, and the photographic properties of the images obtained were studied. The image colours compared with the quinine control were as follows:

| Example No.      | Compound                                    | Image colour                        |
|------------------|---------------------------------------------|-------------------------------------|
| Quinine control. | Quinine bisulphate.....                     | Standard blue.                      |
| 1.....           | 4-methyl quinoline.....                     | Shade less blue than standard.      |
| 2.....           | 6-ethoxy-4-methyl quinoline hydrochloride.  | Similar to standard.                |
| 3.....           | 6-methoxy-4-methyl quinoline hydrochloride. | Bluer than standard.                |
| 4.....           | 4,6-dimethyl quinoline hydrochloride.       | Slightly bluer than standard.       |
| 5.....           | 8-ethoxy-4-methyl quinoline hydrochloride.  | Shade bluer than standard.          |
| 6.....           | 3,4-dimethyl quinoline hydrochloride.       | Distinctly bluer than standard.     |
| 7.....           | 6-ethoxy-3,4-dimethyl quinoline bisulphate. | Trace less blue than standard.      |
| 8.....           | 4,7-dimethyl quinoline hydrochloride.       | Slightly bluer than standard.       |
| 9.....           | 3,4-dimethyl quinoline bisulphate.          | Distinctly bluer than standard.     |
| 10.....          | 3-ethyl-4-methyl quinoline hydrochloride.   | Similar to standard but slate blue. |
| 11.....          | 3,4-tetramethylene quinoline bisulphate.    | Do.                                 |

The solutions of the compounds of the examples were made in ethyl alcohol or water according to convenience. It will be noted that all of the compounds effect a very substantial bluing of the image colour, always comparable with that obtained by the use of quinine, and in some cases even greater than that obtained by the use of quinine. Moreover, the speed loss resultant on the use of the compounds was in no case very serious, and in most cases was not very much different from the speed loss resultant on the use of quinine.

The compounds did not lead to any substantial increase in the fog level of the emulsion, and did not affect the contrast characteristics of the emulsion to any marked extent. All the compounds therefore are very valuable substitutes for quinine.

It is to be understood that in the foregoing description and in the following claims the expression "silver chloride photographic emulsion" means a photographic emulsion in which the predominant silver salt is silver chloride and includes the possibility of a small proportion of other silver halide being present.

What we claim is:

1. Silver-chloride photographic emulsions containing a compound selected from the class consisting of compounds of the general formula:



where R<sub>1</sub> is selected from the class consisting of alkyl, aralkyl and, with R<sub>2</sub> and the two carbon atoms of the heterocyclic ring attached thereto, an alicyclic nucleus; R<sub>2</sub> is selected from the group consisting of hydrogen, alkyl, aralkyl, and, with R<sub>1</sub> and the two carbon atoms of the heterocyclic

clic ring attached thereto, an alicyclic nucleus; R<sub>3</sub> is selected from the group consisting of the hydrogen atom and lower alkyl groups; R<sub>4</sub> is a member of the group consisting of the hydrogen atom, halogen atoms, hydrocarbon, alkoxy, araloxyl, aralkyloxy and a hydrocarbon radical which forms a benzene ring with two adjacent carbon atoms of the carbocyclic ring; and the mineral acid salts of any such compounds.

2. A photographic element comprising a support bearing a gelatino silver chloride emulsion layer containing a compound selected from the class consisting of compounds of the general formula



where R<sub>1</sub> is selected from the class consisting of alkyl, aralkyl, and, with R<sub>2</sub> and the two carbon atoms of the heterocyclic ring attached thereto, an alicyclic nucleus; R<sub>2</sub> is selected from the group consisting of hydrogen, alkyl, aralkyl and, with R<sub>1</sub> and the two carbon atoms of the heterocyclic ring attached thereto, an alicyclic nucleus; R<sub>3</sub> is selected from the group consisting of the hydrogen atom and lower alkyl groups; R<sub>4</sub> is a member of the group consisting of the hydrogen atom, halogen atoms, hydrocarbon, alkoxy, araloxyl, aralkyloxy and a hydrocarbon radical which forms a benzene ring with two adjacent carbon atoms of the carbocyclic ring; and the mineral acid salts of any of such compounds in an amount of the order of 5-50 ccs. of a 1% ethyl alcohol solution per pound of emulsion.

3. Gelatino silver chloride photographic emulsions containing a 4-alkyl quinoline which is unsubstituted in the 2-position and in which the group attached to the carbon atom in the 3-position is selected from the class consisting of the hydrogen atom and alkyl and aralkyl groups.

4. Gelatino silver chloride photographic emulsions containing a 4-methyl quinoline which is unsubstituted in the 2-position and in which the group attached to the carbon atom in the 3-position is selected from the class consisting of the hydrogen atom and alkyl and aralkyl groups.

5. Gelatino silver chloride photographic emulsions containing a 4-alkyl quinoline which is unsubstituted in the 2-position and which contains an alkoxy substituent in the carbocyclic ring and in which the group attached to the carbon atom in the 3-position is selected from the class consisting of the hydrogen atom and alkyl and aralkyl groups.

6. Gelatino silver chloride photographic emulsions containing a 4-methyl quinoline which is unsubstituted in the 2-position and contains a lower alkoxy substituent in one of the 6 and 8 positions and in which the group attached to the carbon atom in the 3-position is selected from the class consisting of the hydrogen atom and alkyl and aralkyl groups.

7. Gelatino silver chloride photographic emulsions containing a 4-alkyl quinoline which is unsubstituted in the 2-position and contains a lower alkyl substituent in the 3-position.

8. Gelatino silver chloride photographic emulsions containing a 4-methyl quinoline which is unsubstituted in the 2-position and contains a lower alkoxy substituent in one of the 6 and 8 positions and a lower alkyl substituent in the 3-position.

9. Gelatino silver chloride photographic emulsions containing a mineral acid salt of a 4-alkyl quinoline which is unsubstituted in the 2-position and in which the group attached to the carbon atom in the 3-position is selected from the class consisting of the hydrogen atom and alkyl and aralkyl groups.

10. Gelatino silver chloride photographic emulsions containing a mineral acid salt of a 4-alkyl quinoline which is unsubstituted in the 2-position and contains a lower alkoxy substituent in one of the 6 and 8 positions and in which the group attached to the carbon atom in the 3-position is selected from the class consisting of the hydrogen atom and alkyl and aralkyl groups.

11. Gelatino silver chloride photographic emulsions containing a mineral acid salt of a 4-alkyl quinoline which is unsubstituted in the 2-position and contains a lower alkyl substituent in the 3-position.

12. A photographic element comprising a support bearing at least one gelatino silver chloride emulsion layer which layer contains a 4-methyl quinoline which is unsubstituted in the 2-position and in which the group attached to the carbon atom in the 3-position is selected from the class consisting of the hydrogen atom and alkyl and aralkyl groups.

13. A photographic element comprising a support bearing at least one gelatino-silver chloride emulsion layer which layer contains a small amount of 6-methoxy-4-methyl-quinoline hydrochloride.

14. A photographic element comprising a support bearing at least one gelatino-silver chloride emulsion layer which layer contains a small amount of 3,4-dimethyl quinoline hydrochloride.

JOHN DAVID KENDALL.  
DOUGLAS JAMES FRY.

**Certificate of Correction**

Patent No. 2,397,015.

March 19, 1946.

JOHN DAVID KENDALL ET AL.

It is hereby certified that errors appear in the printed specification of the above numbered patent requiring correction as follows: Page 2, first column, line 8, for "smulsion" read *emulsion*; and second column, line 13, for "consisiting" read *consisting*; line 55, for "corbon" read *carbon*; page 3, second column, line 8, claim 12, after "groups" and before the period insert *in an amount of the order of 5-50 ccs. of a 1% ethyl alcohol solution per pound of emulsion*; and that the said Letters Patent should be read with these corrections therein that the same may conform to the record of the case in the Patent Office.

Signed and sealed this 28th day of May, A. D. 1946.

[SEAL]

LESLIE FRAZER,  
First Assistant Commissioner of Patents.

9. Gelatino silver chloride photographic emulsions containing a mineral acid salt of a 4-alkyl quinoline which is unsubstituted in the 2-position and in which the group attached to the carbon atom in the 3-position is selected from the class consisting of the hydrogen atom and alkyl and aralkyl groups.

10. Gelatino silver chloride photographic emulsions containing a mineral acid salt of a 4-alkyl quinoline which is unsubstituted in the 2-position and contains a lower alkoxy substituent in one of the 6 and 8 positions and in which the group attached to the carbon atom in the 3-position is selected from the class consisting of the hydrogen atom and alkyl and aralkyl groups.

11. Gelatino silver chloride photographic emulsions containing a mineral acid salt of a 4-alkyl quinoline which is unsubstituted in the 2-position and contains a lower alkyl substituent in the 3-position.

12. A photographic element comprising a support bearing at least one gelatino silver chloride emulsion layer which layer contains a 4-methyl quinoline which is unsubstituted in the 2-position and in which the group attached to the carbon atom in the 3-position is selected from the class consisting of the hydrogen atom and alkyl and aralkyl groups.

13. A photographic element comprising a support bearing at least one gelatino-silver chloride emulsion layer which layer contains a small amount of 6-methoxy-4-methyl-quinoline hydrochloride.

14. A photographic element comprising a support bearing at least one gelatino-silver chloride emulsion layer which layer contains a small amount of 3,4-dimethyl quinoline hydrochloride.

JOHN DAVID KENDALL.  
DOUGLAS JAMES FRY.

**Certificate of Correction**

Patent No. 2,397,015.

March 19, 1946.

JOHN DAVID KENDALL ET AL.

It is hereby certified that errors appear in the printed specification of the above numbered patent requiring correction as follows: Page 2, first column, line 8, for "smulsion" read *emulsion*; and second column, line 13, for "consisiting" read *consisting*; line 55, for "corbon" read *carbon*; page 3, second column, line 8, claim 12, after "groups" and before the period insert *in an amount of the order of 5-50 ccs. of a 1% ethyl alcohol solution per pound of emulsion*; and that the said Letters Patent should be read with these corrections therein that the same may conform to the record of the case in the Patent Office.

Signed and sealed this 28th day of May, A. D. 1946.

[SEAL]

LESLIE FRAZER,  
First Assistant Commissioner of Patents.